

## UNITED STATES PATENT OFFICE.

HIROSHI SHIOKAWA, OF KOBE, JAPAN.

## PROCESS OF TREATING STEEL.

No Drawing.

Application filed August 26, 1922. Serial No. 584,550.

*To all whom it may concern:*

Be it known that I, HIROSHI SHIOKAWA, a subject of the Emperor of Japan, and resident of 18 Nichome, Dainichidori, in the city of Kobe, in the Prefecture of Hyogo and Empire of Japan, have invented a new and useful Process of Treating Steel, of which the following is a specification.

This invention relates to a process of treating steel, more particularly to the treating of shaped steel bodies formed by rolling, forging or in any other manner, and the invention has for its object to provide, in a manner as hereinafter set forth, a process of treating steel bodies to improve the quality and mechanical properties thereof. What is meant by "quality and mechanical properties" is that the body of steel treated by the present process has its quality improved by making it of a uniform structure throughout, and by imparting to it proper degrees of elongation and toughness with a very small loss of tensile strength, and further by driving off the occluded gases therefrom with consequent elimination of undue brittleness, whereby the elongation and toughness are considerably increased while preserving the desirable degree or amount of tensile strength attributable to the elimination of the internal stresses and strains and absorbed gases from the steel body.

The process comprises the conveying the body of steel to a suitable enclosure while the same still retains excess of heat ranging from 500 to 700 degrees centigrade, disposing the same under conditions calculated to prevent said excess of heat from radiating and being lost to no purpose and to produce a uniform temperature throughout its entire mass, causing it to cool very slowly after maintaining said uniform temperature for a certain length of time, and taking it out on its being completely cooled.

The primary object of this invention is to save the cost and time required in the usual reheating system of annealing and to provide an excellent steel body with perfectly uniform structure economically and easily without any loss of qualities of steel incident to said reheating system of annealing.

Other objects and advantages to be derived from the use of this invention will be

apparent from the following detailed description and the claims:

My present invention aims at obtaining a body of steel perfectly uniform in structure and possessing various characteristics economically by treating such body at temperatures lower than the  $A_1$  transformation point (usual annealing temperature) of steel by utilizing the excess of heat retained by it and then causing it to cool slowly, without any resort to the reheating system of annealing hitherto in practice in various countries, and so the process has a very wide range of application with consequent modifications in details of design and practice according to ingredients, sizes, etc., of the body of steel to be treated, and it may be quite clear that those modifications that come within the sphere of the appended claims all fall under the spirit of my invention; but to avoid unnecessary confusion and make the invention easy to understand for one skilled in the art to which it appertains, I will specifically describe the method of applying it to the final or quality treatment of steel plates as an example, thus:

As the first step, a slow-cooling pit is provided at a place convenient for such work and the pit is lined with ordinary brick at the bottom and sides in such a way that loss of heat may be minimized, and then the temperature within the pit is maintained at a height, lower than the  $A_1$  transformation point of steel, suitable for the particular operation to be performed.

At the end of the rolling operation, a steel plate still retains temperatures ranging from 500 to 700 degrees centigrade, and just at this moment the plate is conveyed into the slow-cooling pit prepared in the manner referred to hereinbefore to prevent lowering of its temperature, and another plate is put into and laid on the first one, and so on, until a suitable number of plates are superposed, and finally some lime is spread over the pile; and then a cover or door is placed on the top of the pit and hermetically sealed so as to thoroughly insulate the interior from the atmosphere; and, if said plates are left in this state for 20 to 48 hours or more (length of time being determined by the size and thickness of the steel plate), each plate be-

comes perfectly uniform in temperature throughout its entire length and sectional area, that is, the entire mass, owing to the fact that the excess of heat of the plate is 5 retained in the interior of the pit, and, since suitable amount of energy is imparted to the steel plate, its internal stresses are thoroughly removed, gas or gases previously absorbed in the steel mass are completely 10 driven off, and the entire structure made uniform throughout, and then the plate is slowly cooled, so that there is no possibility for such gas or gases to be re-absorbed or mechanical stresses to reappear, with the result that the qualities and mechanical properties of the finished plate are perfectly normalized and improved. By my improved process, loss of qualities of steel attributable 15 to direct heating at high temperatures as in the case of the usual reheating system of annealing is perfectly eliminated, and, since it does not require any reheating, cost and labor attending to such reheating can be dispensed with, which means a decided advantage 20 over the usual system of annealing. Experiments conducted by me show that a steel plate treated by my improved process possesses an elongation coefficient higher than a similar plate freely cooled in the air by 3 to 8 per cent, and has, in addition, an important feature of being free from breakage 25 or rupture.

As it is necessary to prolong or shorten 30 length of time for maintaining the required uniform temperature and for slow-cooling, so is it needed to adjust time of treatment to meet various requirements, when applying my present invention to bodies of steel other than plates, according as such body is greater or smaller than the plate, which fact may 35 be readily understood. When the articles to be treated are of great bulk, it is often advisable to treat one or a few at a time. In short, it is necessary to modify modes of application, though strictly on the same principle, more or less to adapt the invention to particular needs, which modifications may 40 be done with ease, provided that full understanding of the principle underlying my invention is once obtained.

I am aware that there is a kind of furnace for equalizing the temperature of a steel ingot throughout its entire mass to prepare it for rolling and other operations when its 45 interior is too hot, and another furnace for preparing a cold body of steel or a steel ingot too cold to be rolled at once for such operations by heating it uniformly throughout its entire mass, strictly on the principle of the first-mentioned furnace, as may be inferred from the following quotation from "Iron and Steel" by Erik Oberg and Franklin D. Jones, First Edition, pp. 146 to 147, published by the Industrial Press, New York 50 City:

"Soaking Pits:—As the outside of the ingot cools more rapidly than the inside, the inside may be too hot to be rolled or hammered when the outside is hard. The ingot must, therefore, be brought to a uniform 70 heat, which is done by placing it in the soaking pit. This is a covered brick-lined well in which the ingot is stood on end. It retains the heat of previous ingots, so that the excess of heat in the interior of the ingot placed in it soaks through the mass but is not lost. As a result, the steel is prepared for the mill without the consumption of any fuel. In addition, the waste of iron due to oxidation of the outer crust of ingot is very 80 slight, because the little atmospheric oxygen in the pit at the beginning is not renewed as it is in a furnace. Later forms of soaking pits, however, are heated by regenerative furnaces, so as to give greater flexibility to 85 the system. In one plant the soaking pit consists of four holes, in each of which six ingots may be placed at one time."

Either of the two heat-equalizing furnaces referred to hereinbefore has the sole 90 object of making the steel material fit for rolling and some other operations by treating it at temperatures ranging from 1100 to 1200 degrees centigrade. In other words, either of the two types aims at equalizing 95 the temperature of the steel material under treatment throughout its entire mass, this temperature being much higher than the  $A^1$  transformation point of steel, and it is quite 100 obvious that neither has the least consideration for preventing those strains and internal stresses which may be produced in the steel during the rolling or similar operation or while cooling. And, since it is usual for the steel ingot treated in either type of furnace to arrive at a condition suitable for the 105 intended operation in 20 to 60 minutes, it is also very clear that the furnace is under no condition to cool slowly; on the contrary, its sole purpose is to cool the steel as quickly 110 as possible to render it suitable or to heat it as rapidly as possible to make it suited to said operation. In short, such a furnace is quite different from my present invention, in fundamental principles, which treats steel 115 after it is formed into proper shape to eliminate its defects and impart desirable qualities and mechanical properties thereto.

My present invention differs from either of said two heat-equalizing furnaces or soaking pits in the following essentials:

(1) My present invention has for its object to equalize or normalize qualities and mechanical properties of steel after it is formed, while the furnaces above mentioned treat the steel material itself previous to the forming or shaping operation so as to render such material workable.

(2) My present invention has as one essential condition to equalize the temperature 130

of a steel, semi-manufacture both inside and outside, at a temperature lower than the  $A^1$  transformation point of steel, while the furnaces above mentioned are conditioned to equalize temperature of steel material at a temperature higher than said  $A^1$  transformation point.

(3) My present invention aims at imparting effects similar to or even superior to those obtained by the usual system of annealing, by causing temperature of the steel body throughout its entire mass to equalize at about 400 to 500 degrees centigrade and then maintaining this uniform temperature for a certain length of time, while the furnace has the sole purpose of rendering steel material itself suitable for working or shaping operation in as short a time as possible.

From the said three items, it is as clear as day that my present invention is quite different from the furnace both in principle and objects, and there may be no room for the least doubt. Though the slow-cooling pit referred to hereinbefore as an example of practice of my present invention is somewhat similar to the soaking pit in form, yet with my invention the slow-cooling pit is nothing but a means of practising the principle underlying the same, and utilization of the excess of heat and improvement of the qualities and mechanical properties at temperatures lower than the  $A^1$  transformation point of steel are quite different from the object of the heat-equalizing furnace, and it will be readily seen that my invention is utterly independent of said furnace.

The novelty and utility of my present invention will be understood more definitely and clearly, by comparing the same with various kinds of heat-treatments of steel hitherto in use. To be precise in this connection, I shall quote the following definitions from "Engineering Steels" by Leslie Aitchison, pp. 39, published by Macdonald & Evans, London, thus:

(1) "Normalizing.—Normalizing means heating a steel (however previously treated) to a temperature exceeding its upper critical range, and allowing it to cool freely in the air.

(2) "Annealing.—Annealing means reheating, followed by slow cooling. Its purposes may be:

(a) To remove internal stress, or to produce softness, in which cases the maximum temperature may be arbitrarily chosen.

(b) To refine the crystallized grains in addition to the above (a), in which case the temperature used must exceed the upper critical range as in normalizing.

(3) "Hardening.—Hardening means heating a steel to its normalizing temperature, and cooling more or less rapidly in a suitable medium, e. g., water, oil, or air.

(4) "Tempering.—Tempering means heat-

ing a steel (however previously hardened) to a temperature below its carbon change-point, with the object of reducing the hardness or increasing the toughness to a greater or less degree.

(5) "Softening.—Softening is to facilitate the machining of a steel, and is carried out by annealing or tempering, or both."

(A) Difference between my invention and normalizing: The object of normalizing is to remove stresses, strains or similar abnormal state produced within the steel while the same is undergoing rolling, hammering, drop-forging, casting and other operations. Though it may be considered that this heat-treatment resembles my present invention in some respects, yet the former has for its condition to reheat steel, previously treated, to a temperature exceeding the upper critical range and then to cool it freely in the air, while the latter is conditioned to treat a steel body at a temperature lower than the lower critical range and then to cause it to cool slowly in the slow-cooling pit insulated from the outer air, and so it is quite obvious that the two processes differ fundamentally from each other from the viewpoint of metallurgy, to say nothing of the fact that the latter has a special feature of attaining the object economically by utilizing excess of heat of the article under treatment.

(B) Difference between my invention and annealing: Annealing aims at removing internal stresses or refining the crystalline structure in addition to said removal of internal stresses. When removal of internal stresses alone is the object aimed at, the maximum temperature may be arbitrarily decided, but, when removal of internal stresses and the improving of the structure of the crystallized grains are to be accomplished at once, treating the steel at a temperature exceeding the upper critical range is an essential condition. In either case, reheating of the steel manufacture or product to a certain temperature is absolutely necessary. My present invention may seem to resemble somewhat annealing in the results obtained, but in the fundamental principles and modes of operations both differ much, as may be seen from the following statement:

(1) Difference between my invention and annealing having its sole object to remove internal stresses:—(a) My invention has a special feature of improving qualities and mechanical properties of the steel manufacture or semi-manufacture treated economically by utilizing the excess of heat of the article itself, while the latter process has the defect of requiring reheating with consequent loss of time and labor as well as fuel.

(b) With my invention, the temperature at which to treat the steel body is limited to

a range of 400 to 500 degrees centigrade for uniformity and said temperature is obtained automatically, so that any person can practise it with ease and security of results, 5 while in the latter process the maximum temperature is not certain with consequent difficulty of determining the suitable temperature for a particular article to be treated, in addition to the fact that good results 10 can be obtained by skillful persons alone. (c) My invention can accomplish the double object of removing internal stresses and improving the structure of the crystallized grains by one operation, but the latter can 15 only remove internal stresses or to soften the steel.

(2) Difference between my invention and annealing aiming at removal of internal stresses and refining of crystalline structure 20 at once:—(a) My invention has the advantage of being able to improve qualities and mechanical properties of steel product economically by utilizing the excess of heat of the product itself, but the latter process requires reheating with consequent waste of fuel, time and labor. (b) My invention is conditioned to treat steel at a temperature lower than the  $A^1$  transformation point of 25 steel, while the latter process is required to treat steel at a temperature exceeding said transformation point. (c) My invention has a special feature of being able to eliminate 30 defects alone and to retain useful qualities at the same time owing to the fact that no reheating is needed to impair qualities of steel, but in the latter process it is essential to 35 reheat the steel to a temperature exceeding the upper critical range with consequent result that the steel is transformed more than is really required, producing loss of some 40 of the desirable properties and impairment of the steel due to direct heating.

In a word, the fundamental difference between my invention and annealing lies in 45 the fact that in my invention the excess of heat is utilized to accomplish the objects in view, and that treatment of the steel body is carried out with better results than those of the reheating system of annealing, at a 50 temperature lower than  $A^1$  transformation point of steel; in other words, my invention combines novelty and utility which cannot be found in the annealing process.

(C) Difference between my invention and 55 tempering: The object of tempering is to heat the steel to a temperature lower than the carbon-change point ( $A^1$  transformation point), when the steel previously hardened has been completely changed to solid solution, which is especially the case with special 60 steels, and become too hard and brittle, to render it softer or a little tougher, and the treatment may seem to have some points in common with my invention at first thought, 65 but on closer observation it will be readily

found that they differ remarkably in the following respects:

(a) My invention has as one of its conditions to utilize excess of heat of the steel under treatment, while the latter requires 70 reheating.

(b) My invention has as its object to remove internal stresses and improve qualities and mechanical properties of the steel treated, while the latter aims at changing the 75 steel from solid solution to mixture of ferrite and pearlite to reduce its hardness, a very remarkable difference.

(c) My invention has an advantage of 80 treating steel at a suitable temperature and then slowly cooling it so as to enable the treated article to retain its desirable qualities imparted thereto by the low-temperature treatment, while in tempering no slow-cooling is employed, and it is clear that they 85 differ in this point, too.

(d) Since the temperature for treatment is limited to from 400 to 500 degrees centigrade in the case of my invention, there is no need of special care and trouble in this 90 respect, while in tempering the treating temperature occupies a very wide range from room temperature to that slightly lower than the  $A^1$  transformation point with consequent trouble and drawbacks for 95 practical purposes.

In short, my invention combines the three conditions of (1) accomplishing the desired results economically by utilizing the excess of heat, (2) of rendering determination of 100 the suitable temperature for treatment extremely simple, and (3) of enabling the article treated to retain desirable qualities and characteristics, while tempering possesses none of said three features, and it will 105 be readily seen that there is a fundamental difference between these two processes, and that my invention has perfect novelty and utility quite independent of the tempering.

(D) Difference between my invention and 110 softening: Softening is a kind of heat-treatment aiming at rendering steel easy to machine, and is carried out by either annealing or tempering, or by both. The difference between my invention and annealing 115 and that between my invention and tempering have been treated in detail hereinbefore, and so the difference between my invention and softening may be quite clear 120 without any further explanation.

The above-mentioned specific description is enough, I believe, to give one skilled in the art to which it appertains a full understanding of my present invention, and to prove the fact that my invention has novelty 125 and utility quite independent of any of the said kinds of heat-treatments.

Having thus fully described my invention, what I claim as new and desire to secure by 130 Letters Patent, is:

1. A process of treating steel comprising the placing of a body of rolled or forged steel while it still retains an excess of heat remaining after the working operation, at 5 a temperature below the transformation point in a hermetically sealed enclosure free of direct heating for said body, then allowing said body to remain in said enclosure for a predetermined period to utilize such excess heat at a uniform temperature to remove internal stresses and gases from said body to provide a uniform structure throughout, and further for the slow cooling of said body.
- 15 2. A process of treating steel comprising the placing of a body of rolled or forged steel while it retains an excess of heat remaining after the working operation ranging from 500 to 700 degrees centigrade in a 20 hermetically sealed enclosure for a predetermined period to equalize such excess of heat at a uniform temperature to remove internal stresses and gases from said body to provide a uniform structure throughout, 25 and then slowly cooling said body in said enclosure.
- 30 3. The process of improving qualities and mechanical properties of a rolled or forged steel body consisting in conveying the same, while it still retains an excess of

heat remaining after the working operation ranging from 500 to 700 degrees centigrade, into a slow-cooling pit previously kept at a temperature higher than 400 degrees centigrade but lower than 700 degrees centigrade until suitable quantities of such bodies are reached, spreading lime over the upper layer or portion at the end of said conveying operation, then insulating the interior of said pit from the outside air so as to equalize the temperature of said bodies at about 400 degrees centigrade throughout the entire mass, and finally causing the same to cool slowly, substantially as and for the purposes set forth. 35 40 45

4. A process of treating steel comprising the conveying of a body of rolled or forged steel, while it retains an excess of heat remaining after the working operation ranging from 500 to 700 degrees centigrade, into 50 a cooling pit at a temperature lower than 700 degrees centigrade, then spreading a covering of lime over said body, then providing for the equalizing of the temperature throughout said body to about 400 degrees centigrade, and then slowing cooling the body within the pit. 55

In testimony whereof I affix my signature hereunto.

HIROSHI SHIOKAWA.